

# UNITED STATES PATENT OFFICE.

JAMES W. NEILL, OF SALT LAKE CITY, UTAH.

## METHOD OF LEACHING COPPER ORES.

SPECIFICATION forming part of Letters Patent No. 650,784, dated May 29, 1900.

Application filed September 29, 1899. Serial No. 732,111. (No specimens.)

*To all whom it may concern:*

Be it known that I, JAMES W. NEILL, a citizen of the United States, residing at Salt Lake City, in the county of Salt Lake and State of Utah, have invented certain new and useful Improvements in Methods of Leaching and Extracting Copper Ores; and I do hereby declare the following to be a full, clear, and exact description of the invention, such as will enable others skilled in the art to which it appertains to make and use the same.

My invention relates to the extraction of copper from ores or tailings of copper ores or other materials containing copper.

15 The process forming my invention is applicable to some ores in their natural state without a preliminary roasting of the same, although in other cases—as, for instance, in the case of the sulfid-of-copper ores—a preliminary roasting of the ore is necessary. Inasmuch as my invention has its chief field of usefulness in the extraction of copper from sulfid-of-copper ores the process will be described more particularly in its application to 20 ores of that character.

25 The object of the process, as usual in the art, is to finally obtain the copper contained in the ore in a metallic state, or as cupric oxide, or as cuprous sulfid, or in other commercial form; but the main or principal features of the process which constitute my invention are, briefly, first, the subjection of the ores (either with or without previous roasting of the same, depending upon the 30 character of the ore) to the action of sulfurous acid (as gas or in solution) to dissolve out the copper, and, second, the heating of the solution thus obtained to drive off the excess of sulfurous acid and form a copper precipitate, which may be subjected to any desired after treatment or not, as may be required.

35 In the case of sulfid-of-copper ores or other ores containing sulfur as a constituent the roasting of the ore has the incidental advantage that it affords as a by-product the sulfurous acid employed in my process. In other cases the sulfurous acid may be obtained from the direct burning of sulfur or in other 40 ways, as well understood in the art. I am aware that sulfuric acid has been very commonly employed in the extracting of copper

from its ores; but the advantages in the use of sulfurous acid are very many. Sulfuric acid can seldom be bought in localities where 55 copper ores abound at less than two cents per pound, and in such localities “roast fumes” are usually abundant, and my solvent sulfurous acid would practically cost nothing; but were there no “roast fumes or gases” 60 and if it were necessary to use sulfur instead my method of treatment of ores or tailings, above referred to, is still much cheaper. In places where sulfuric acid can be bought for two cents per pound sulfur can also be bought 65 for two cents per pound. It takes ninety-eight pounds of sulfuric acid to dissolve sixty-three pounds of copper, while it only takes thirty-two pounds of sulfur in the form of sulfurous acid to dissolve the same amount 70 of copper—sixty-three pounds. Therefore my method in this case is three times as cheap in the cost of material used in treating material and ores, above referred to, containing copper, as compared with sulfuric acid; but the 75 advantage flowing from the use of sulfurous acid does not stop there. It (sulfurous acid) being a much weaker acid than sulfuric acid, does not attack so vigorously the other metallic contents contained in the ores or material treated, thus fouling the solution and wasting the acid. Neither does it (sulfurous acid) attack the vessels or implements of the plants to the same extent as the stronger acid (sulfuric) would do, and for the same 80 reason it is much easier and cheaper to reduce the copper obtained from the ores and tailings after treatment with sulfurous acid than it would be to reduce the copper obtained by sulfuric acid, either by using the 85 electric current or scrap-iron.

90 The sulfurous acid as employed in my process may be used either as a gas (as will be presently described) or in solution, or both, at atmospheric pressure. When my process 95 is applied in the extraction of copper from sulfid-of-copper ores and other similar ores or materials hereinafter named, the ore is first roasted, having been previously crushed (preferably when dry) so as to pass a suitable-sized screen-mesh. The effect of this roasting is to convert the copper sulfids, as far as may be, into copper oxids. This roasting operation does not need to be a “dead roast;” 100

but preferably the sulfur contents of the ore, tailings, or material after the roasting should contain sulfur below one per cent., (1%).) Then and in that case the copper is entirely soluble in sulfurous acid, and my process is thus best carried out. The ore is now ready to be subjected to the action of sulfurous acid, (as gas is in solution,) which constitutes the first step of my improved process. This may be accomplished by placing the crushed and roasted ores in tanks or vats, preferably of wood and of a size and shape adapted to special or local conditions. These vats or tanks may be supplied with stirring-arms or other devices by which to agitate the contents, and thus hold the ores in a state of suspension, or the vats may be only supplied with false bottoms and filtering-cloth. In these vats the ore is subjected to the action of sulfurous-acid solution or of sulfurous-acid gas, or both, direct, and the ores may be kept in a state of suspension, if desired or necessary, or may be allowed to remain in place in the tanks or vats, and the solution or gas may then be percolated through the mass of the ore. As soon as the copper is dissolved by the solution or the gas, and this may be easily determined by taking a small sample from the tank or vat and testing it in the usual manner for copper, the solution is then withdrawn from the ore either by filtration, allowing the previously agitated mass to settle, then decanting the solution, or by other means, and this solution I pass to other vats for further manipulation. The ore is then preferably given a washing with pure water or water containing a small amount of sulfurous acid in order to remove any of the solution carrying the copper, and so clean out the ore and leave it in a condition where it may be taken from the tanks or vats and thrown on a dump as a waste. This washwater may be saved and used in the apparatus for collecting and making the solution of sulfurous acid and reused as a solvent on the ore, thus making a saving of water in districts where the same is scarce. The solution of sulfurous acid containing copper, as cuprous sulfite, held in solution therein by the excess of sulfurous-acid gas, is now subjected to the second step of my improved process, which consists in heating the solution to a temperature sufficient to drive out the excess of sulfurous acid, thereby precipitating the copper in the form of a bright-red and very heavy powder, (cuprous sulfite.) This cuprous sulfite settles at once to the bottom of the tank or vat, and the remaining solution may be readily and entirely siphoned or decanted from it, or the cuprous sulfite may be recovered from the solution by filtration. To effect the heating or boiling of the solution, waste or exhaust steam may be used while the solution is contained in wooden tanks or vats, thus making it a very cheap method of extracting copper from the solution. The excess of sulfurous-acid

gas thus driven out of the solution may be carried to the apparatus and again absorbed in water, thus preventing any losses or escape of gas. The cuprous sulfite after it has been removed from the tanks or vats, filtered, and dried contains about fifty per cent. of metallic copper, and it may be heated in an oxidizing atmosphere in a furnace and the cupric oxide produced, which is useful in commerce and may be sold as such, or it may be melted in a furnace in a reducing atmosphere, producing cuprous sulfid, which may then be reduced to metallic copper in the process known as the "Bessemer" process, for which this material would be perfectly fitted.

Should the oxidation or roasting of the crude ore not have been perfect, some copper sulfate will remain in the ore and be taken up by the solution. In this case all the copper will not be precipitated by boiling of the solution, and some will remain in the residual solution. This must be either passed over scrap-iron to regain this remaining portion of copper, or it may be passed through vats, where it is subjected to the action of an electric current, which precipitates the copper.

The sulfurous acid used in the above process to dissolve the copper from the ore may, as already stated, be obtained from any desired source. Preferably I obtain it from the sulfid ore by collecting the fumes from the roasting-furnaces. These may be passed through water in some well-known and usual manner in a suitable apparatus, such as tanks or towers of wood or stones over which water is allowed to drip, the sulfurous-acid gas being absorbed by the water and this hydrated sulfurous acid so made being used as the solvent for dissolving copper from its ores or tailings. It is very apparent that this solvent thus made is a very cheap one and, furthermore, that the absorption of this harmful gas from the furnace-fumes must be a great benefit to a community around metallurgical works where this gas is produced. In other cases or under other conditions the sulfurous acid (gas) obtained in the manner above stated or in any other manner may be applied to dissolve out the copper by passing it at once through vats containing the ores (oxids or carbonates) in a state of pulverization and wet, the ore suspended by continued agitation in the water, if so desired or expedient, or the gas may be caused to ascend through a mass of the wet ore, which dissolves the copper therefrom very rapidly, and the salt so formed is at once taken up by the water and held in solution.

My process may also be applied to ores in which the copper is present naturally in the form of an oxid of copper, as in cuprite, or when the copper is present in the form of a carbonite of copper, as in malachite or azurite. When the copper is present as sulfid chalcopyrite, chalcocite, bornite, &c., the copper ore must first be converted into the form of

an oxid by roasting same, as hereinbefore described, and then dissolved from the ore by means of the sulfurous-acid gas or a solution of the gas or both.

5 In the foregoing specification and following claims the term "ore" is used as including tailings or other material or ore treated by roasting or otherwise previously to treatment by my process.

10 Having described my invention, what I claim, and desire to secure by Letters Patent, is—

15 1. The herein-described process of extracting copper from copper ores consisting in first dissolving out the copper by means of sulfurous acid and then heating the resultant solution to drive off the excess of sulfurous acid and precipitate the copper as and for the purpose described.

20 2. The process of treating and extracting

copper from sulfid-of-copper ores, tailings or material containing sulfid of copper, consisting in roasting the ore in the presence of air, thereby oxidizing and liberating the sulfur therein combined, thus forming sulfurous- 25 acid gas, collecting the product of combustion and oxidation in water, thus forming sulfurous acid, dissolving the copper contained in the burned ore by means of the solution obtained from the water and product of combustion and oxidation and precipitating the copper from the resultant solution by heating the same.

In testimony whereof I have hereunto affixed my signature in presence of two wit- 35 nesses.

JAMES W. NEILL.

Witnesses:

HENRY STERN,  
JAMES R. ROGERS.